

Sept. 20, 1932.

W. P. WITHEROW

1,878,054

DIE ROLLING AND ARTICLE PRODUCED THEREBY

Original Filed Feb. 7, 1925 2 Sheets-Sheet 1



Fig.1.



Fig.2.



Fig.3.



Fig.4.



Fig.5.



INVENTOR  
William P. Witherow,  
By *James Brown, Parmiter,*  
*an Atty.*

Sept. 20, 1932.

W. P. WITHEROW

1,878,054

DIE ROLLING AND ARTICLE PRODUCED THEREBY

Original Filed Feb. 7, 1925 2 Sheets-Sheet 2

Fig. 8.



Fig. 7.



Fig. 9.



Fig. 10.



Fig. 11.



Fig. 12.



Fig. 13.



Fig. 14.



INVENTOR  
William P. Witherow,  
Bymer, Edwards, Parmely,  
Inc. ators.

## UNITED STATES PATENT OFFICE

WILLIAM P. WITHEROW, OF PITTSBURGH, PENNSYLVANIA, ASSIGNOR, BY MESNE ASSIGNMENTS, TO REPUBLIC STEEL CORPORATION, OF JERSEY CITY, NEW JERSEY, A CORPORATION OF NEW JERSEY

## DIE ROLLING AND ARTICLE PRODUCED THEREBY

Application filed February 7, 1925, Serial No. 7,470. Renewed May 25, 1932.

The present invention relates broadly to metal working, and more particularly die rolling for the production of shapes adapted to be sold as articles of manufacture, or adapted 5 to have a forming or machining operation performed thereon in order to produce finished products.

Heretofore in the art of die rolling it has been customary to select more or less arbitrarily the leader from which the die rolled blanks are to be produced, it having ordinarily been considered of importance only to provide a leader having a sufficient cross section to properly form the desired blanks.

15 In my co-pending application, Serial No. 530,640, filed January 20, 1922, I have disclosed and claimed a method of die rolling comprising utilizing a leader having a major and a minor axis. I have found that a leader 20 having a major and a minor axis is of decided advantage in that it facilitates the die rolling operation and improves the character of the blank produced.

Heretofore, for the successful die rolling 25 of articles, arrangement has been made for the production of a substantial amount of flash, such flash facilitating the reduction to be effected on the leader and assisting in the rolling of blanks to accurate dimensions within the close tolerances permitted. It will be apparent, however, that this flash must necessarily be trimmed before the blanks can be used, and that the amount of waste metal is directly proportional to the amount of flash.

35 The present invention has for one of its objects the provision of a leader by means of which the amount of flash may be materially reduced and the production of blanks facilitated.

40 It has heretofore been considered necessary in substantially all die rolling operations to provide die rolls with grooves or matrix portions of varying dimensions determined by the shape of the blank to be produced thereby. 45 Ordinarily, such matrix portions have been of a character to produce uniform reduction circumferentially of an article in the event of circular shapes, and usually to produce reduction both vertically and transversely relative of the shapes being rolled. While this

operation is perfectly feasible and practicable for certain shapes, I have found that for other shapes such an operation is exceedingly hard on the rolls, the reduction not being equal throughout the entire length of the 55 blanks and imposing unequal wear on the matrix portions of the grooves at different points. Furthermore, the formation of the rolls is expensive due to the fact that the grooves must necessarily be formed throughout, due to their varying dimensions, on a die sinking or other similar machine.

The present invention has for further of its objects a method of die rolling by means of which the length of life of the rolls is increased and the cost of the rolls is materially decreased and in which substantially all of the reduction is effected in a plane substantially normal to the axis of rotation of the 60 rolls.

In the accompanying drawings I have shown for purposes of illustration only certain preferred embodiments of the present invention, it being understood that the drawings do not define the limits of my invention and that changes in the construction and operation disclosed therein may be made without departing either from the spirit of the invention or the scope of my broader 75 claims.

In the drawings:

Figure 1 is an outline illustrating the configuration of a leader adapted for the formation of a blank such as shown in Figures 2 and 3;

Figure 2 is a side elevation of a cam shaft blank produced in accordance with the present invention;

Figure 3 is a top plan view of the blank shown in Figure 2;

Figure 4 is a transverse sectional view on any of the lines IV-IV of Figures 2 and 3;

Figure 5 is a transverse sectional view on any of the lines V-V of Figures 2 and 3;

Figure 6 is an end elevation of a portion of a pair of rolls adapted for the production of a horse shoe blank;

Figure 7 is a side elevation illustrating a connected series of blanks produced by the rolls shown in Figure 6;

Figure 8 is an end elevation of the blank shown in Figure 7;

Figure 9 is a side elevation of a die rolling blank adapted for the formation of front axles of automotive vehicles;

Figure 10 is a top plan view of the blank shown in Figure 9;

Figure 11 is a transverse sectional view along any of the lines XI—XI of Figures 9 or 10;

Figure 12 is a transverse sectional view along any of the lines XII—XII of Figures 9 or 10;

Figure 13 is a transverse sectional view along any of the lines XIII—XIII of Figures 9 or 10; and

Figure 14 is an outline similar to Figure 1 illustrating a form of leader adapted, for example, for the production of a steering 20 knuckle in accordance with the present invention.

The present invention is distinguished from the prior art among other things by reason of the fact that substantially any section taken through a blank produced by die rolling in accordance herewith is substantially rectangular irrespective of the shape of the transverse section of the finished article to be produced therefrom as contrasted 25 from the generally circular shape heretofore frequently imparted to blanks by the die rolls. It has been found that in this manner the percentage of flash produced can be materially reduced while simplifying the die 30 rolling operation.

The present invention is further characterized by the production of a blank of substantially constant width, the variations being only in a vertical direction, or direction lying 35 in a plane normal to the axis of rotation of the rolls. The leader utilized will also approximate a rectangle as a limit, the leader having a major and a minor axis.

The major axis representing the height of 40 the blank is preferably slightly in excess of the height of the rolled blank to provide the necessary draft and the width of the leader is preferably substantially equal to but slightly less than the width of the rolled blank.

50 The percentage of reduction effected by the die rolls, hereafter designated as R, is determined by the formula:

$$\frac{LA - SA}{LA}$$

in which LA is equal to the large area or normal area of the leader and SA is equal to the smaller area at the point at which the 60 percentage of reduction is to be determined. The area of the flash will be designated FA. In carrying out the present invention the value of FA varies according to R in rolling a leader in which H is the height of the leader 65 and W is the width.

In practicing the present invention the following relations preferably exist:

$$\begin{aligned} H &> W \\ H &> h \\ W &< \text{or } = w \\ H:W::1.5 \text{ to } 3:1 \end{aligned}$$

In the foregoing, *w* represents the average width of the die rolled blank and *h* the maximum height of the die rolled blank at any point.

Referring specifically to Figure 1 of the drawings there is disclosed the transverse outline of a leader which has been found to be highly successful for use in the die rolling 80 of cam shafts and particularly cam shafts of the character suitable for the production of finished cam shafts for a standard automobile. Such a leader has a width slightly less than  $1\frac{1}{2}$  inches and a height slightly less than 85 3 inches, it having been found that very desirable results are produced where W equals  $1\frac{7}{16}$  inches and H equals  $2\frac{3}{4}$  inches. With such a leader the blank shown in Figures 2 and 3 and in cross section in Figures 4 and 5 can be effectively produced. In actual practice, it has been found that with a finished trimmed weight for the blank of 15.6 pounds the total weight of the flash will not exceed 1 pound or slightly more than 6 90 per cent of the weight of a complete blank, this being materially less than it has heretofore been possible to produce in the ordinary practice of die rolling.

Referring to Figure 5 in which the maximum height of the die rolled blank is shown, *h* preferably equals  $2\frac{5}{8}$  inches, this being slightly smaller than *H*, and *w*, representing the average width of the die rolled blank, is  $1\frac{1}{2}$  inches, this being slightly greater than *W*. This blank satisfies the following formulae:

$$\begin{aligned} W &< \text{or } = w \\ H &> W \\ H &> h \end{aligned}$$

It will be noted that the configuration of the leader shown in Figure 1 approaches a rectangle as a limit, the leader, however, having slightly rounded ends 2 and flat sides 3. I believe that in using a leader of this character one reason for the small amount of flash is directly attributable to the substantially straight sides, in which the metal is not initially so disposed as to facilitate lateral flow. The rounded portions 2 on the leader representing the top and bottom thereof are desirable as they improve the draft and also conform approximately to the finished contour 2' of the top and bottom of the die 110 rolled blank as shown in Figures 4 and 5. By keeping these portions slightly curved, the use of sharp corners is entirely obviated and the matrix portions of the die rolls are more completely filled. In the blank, the 115 enlarged portions 4 provide sufficient stock 120

for the subsequent finishing by forging or otherwise of the cams while the smaller portions 5 are adapted to form the bearing portions of the cam shaft. From an inspection 5 of Figure 3 as compared to Figure 2 it will be seen that the die rolled blank is of substantially constant width but of varying height at different portions. In this particular example, the percentage reduction on 10 opposite sides of a median plane passing transversely through the blank from side to side is uniform, the work being distributed equally between the rolls.

I have also found that in carrying out the 15 present invention very desirable results are obtained where the side walls 6 of the die rolled blank converge upwardly and downwardly from an intermediate plane, this plane in the form of the invention shown in 20 Figures 2 to 5 being a median plane through the blank. In Figure 4 the angle of convergence is designated AC, this angle being approximately  $7^{\circ}$ . In Figure 5 the corresponding angle is designated 25  $ac$ , this angle in this instance being approximately  $4^{\circ}$ . It will be noted that the angle of convergence decreases as the value of  $h$  increases, it having been found from actual practice that with such a construction it is possible to obtain a better filled 30 blank and at the same time provide a blank which frees itself more readily from the die rolls.

In Figures 6, 7 and 8 there are shown different features of the invention applicable to the production of a horseshoe blank. In this embodiment of the invention the lower roll 8 has a matrix groove 9 herein shown as being of constant depth and preferably of 35 constant width throughout the entire periphery of the roll. The upper roll 10, however, has a matrix groove 11 of varying dimensions as to depth throughout the periphery of the roll but preferably of substantially constant width, the direction of rotation of the rolls being indicated by the arrow A. These rolls are adapted for the production of the blank shown in Figures 7 and 40 8, in which the blank is of substantially constant width, the base 12 being formed in the matrix groove 9 of the bottom roll and lying in a common plane while the upper portion is formed by the matrix groove 11 in the upper roll. The flash formed during the rolling 45 operation is designated F, this flash being most pronounced adjacent the portions of smaller cross sectional area where the value of R increases. By reference to Figure 8 of the drawings it will be noted that the blank is of substantially constant width, Figures 7 and 50 8 showing that the reduction is effected vertically, or in a plane substantially normal to the axis of rotation of the rolls.

In Figures 9 to 13 there is illustrated another embodiment of my invention in which

the die rolled blank 14, such as adapted for the production of an automobile front axle, has a substantially constant width but varies symmetrically as to height on opposite sides of a median plane. In Figure 12 there is 50 illustrated the minimum cross sectional area of the die rolled blank, this area representing a reduction in actual practice of substantially 69 per cent, the value of  $h$  being substantially  $\frac{7}{8}$  inch in this section as compared to  $2\frac{3}{16}$  inches in Figure 13 which represents the maximum section in which, however, there has been a reduction preferably of approximately 20 per cent for draft purposes and insuring proper formation of the blank. In 55 Figure 12 AC equals substantially  $7^{\circ}$  while  $ac$  in Figures 11 and 13 equals approximately  $4^{\circ}$ . It is not essential that the value of the angle of convergence vary directly as the value of  $h$  varies, but I have found that in most cases this angle should not be materially less than  $4^{\circ}$  and need not be materially greater than  $7^{\circ}$  although this latter figure may be increased materially if desired.

In Figure 14 there is illustrated the configuration of another leader in which  $H$  may equal, for example,  $4\frac{5}{8}$  inches and  $W 2\frac{1}{4}$  inches, it being desired to produce from this leader a blank in which  $w$  shall be equal to substantially  $2\frac{3}{8}$  inches and in which the maximum value of  $h$  is  $4\frac{1}{8}$  inches. This condition also fulfills the following formulæ:

$$W < \text{or } = w$$

$$H > h$$

$$H > W$$

It is not essential in the carrying out of the present invention that the sides of the blank shall lie in parallel planes, it being possible to slightly curve the same while retaining certain of the advantages of the invention. In all cases, however, the radius of curvature of the sides should be greater than the radius of curvature of the ends or the top and bottom of the leader and the leader should have a major and a minor axis. Preferably also the die rolled blank will have a substantially constant width whereby the percentage of flash is materially reduced and the shaping of the article facilitated.

By practicing an invention in which substantially all of the reduction is accomplished in a plane normal to the axis of rotation of the rolls, it will be apparent that it is possible to utilize matrix grooves in the rolls having a substantially constant width. This permits the rolls to be initially placed in an ordinary lathe by means of which a groove is turned therein having a width substantially equal to the desired width of the finished matrix portion and having a minimum depth substantially equal to the minimum depth of such matrix portion. Thereafter the sides of the groove may be ma-

chined or otherwise finished and the bottom of the groove further machined to impart the desired depth thereto. This formation of the major portion of the groove in the lathe or similar machine, as contrasted to the usual process of forming the same in a die sinking machine or die routing indicator represents a material saving not only in time but also in investment. I have also found that by filleting all of the corners, and curving the bottoms of the grooves in both rolls, when combined with the diverging wall relationship to give the desired angle of convergence in the finished blank, crushing down of the rolls is prevented and the length of life materially increased.

The advantages of the present invention arise from a method of die rolling resulting in decreased cost, increased length of life of the die rolls and a decrease in the percentage of flash.

I claim:

1. A die rolled blank having a substantially constant width and having at least a portion of the side walls converging upwardly, the blank being of varying height at different portions and having an angle of convergence decreasing as the blank increases in height.
2. A die rolled blank having a substantially constant width and having at least a portion of its side walls converging downwardly, the blank being of different height in different portions thereof and having an angle of convergence decreasing as the blank increases in height, substantially as described.
3. The method of die rolling, comprising utilizing a uniform leader of quadrangular section having curved top and bottom walls and producing therefrom a blank having a substantially rectangular cross section at any point, said blank being of varying cross section along its length, substantially as described, whereby the production of flash and the wear on the rolls is reduced.
4. The method of die rolling, comprising utilizing a uniform leader having curved side walls of a greater radius than the top and bottom walls and producing therefrom a blank of substantially rectangular cross section at any point, the blank being of varying cross section along its length, substantially as described, whereby the greatest reduction occurs in a plane perpendicular to the roll axis.
5. The method of die rolling, comprising supplying a leader of quadrangular section and having curved top and bottom faces, to a die rolling pass, reducing the leader in all parts in the pass so as to form a blank having a substantially rectangular cross section at any point, the cross sectional area of the blank differing at different parts thereof, there being flash along the sides of the blank in at least certain portions thereof, substan-

tially as described, whereby the maximum reduction is effected in a plane perpendicular to the roll axis.

In testimony whereof I have hereunto set my hand.

WILLIAM P. WITHEROW.